

## UNITED STATES PATENT OFFICE

1,977,932

## COATING COMPOSITION

William Howard Wright, Schenectady, N. Y., assignor to Schenectady Varnish Company, Inc., Schenectady, N. Y., a corporation of New York

No Drawing. Application May 2, 1934,  
Serial No. 723,614

18 Claims. (Cl. 91—70)

The present invention relates to varnishes and enamels and particularly those known to the trade as "wire enamels". Wire enamels are usually applied to wire in a continuous operation by passing the wire through a bath of the enamel and then through a baking chamber, where the coating is dried and baked upon the wire.

Wire, for example, copper wire so coated, is particularly useful in the electrical arts, i. e. in the manufacture of coils for transformers and motors, the coating being of course insulating.

For the purpose of electrical conductors, the wire is usually given a further coating with an insulating varnish and it is necessary that the wire enamel undercoat be resistant to the solvents used in such superposed insulating coatings, as well as be resistant and inert to the wet varnish of this supplemental coating until the latter has become thoroughly dried and baked out.

Furthermore, the wire enamel coating must be resistant to various oils which have a solvent action, such as the cooling oils customarily employed in connection with transformers which frequently reach a high temperature.

Usually the wire enamel is of a type to impart a definite color to the wire. In some cases, a purple, mahogany, or other desired color is obtained, due to the nature of the enamel, the chemical action which takes place between its ingredients, and/or the use of the required baking temperature.

It has also been customary in making so-called "colored enamels", to add a suitable pigment to the enamel to give the desired color such as red, green, yellow, etc., the pigment being suitably ground and the wire enamel acting as a vehicle.

It will be appreciated, therefore, that the manufacture of wire enamels comprehends a number of problems which must be carefully considered and the present invention briefly stated utilizes a solvent which very materially assists in obtaining a hard, smooth, non-porous and flexible coating thoroughly adherent to the metal wire base and offering a maximum of resistance to the action of solvents and temperature conditions.

The manufacture and use of wire enamels entails specific problems in order that a coating of the above desired characteristics will be produced. For example, the constant running of a wire through a bath has a tendency to produce a gelling of the enamel and thereby lower its coating efficiency. This difficulty I find is very considerably relieved by reason of the present invention employing a novel solvent for the enamel.

Also, in the manufacture and use of wire

enamels great care must be exercised to prevent formation of bare spots constituting faults, and likewise a uniform coating must be produced. The enamel of the present invention remains sufficiently fluid both in the bath and in the baking oven, so that up to the time of final setting of the coating, the composition is flowable and thereby self-sealing. In other words, the relatively slow evaporative quality of the coating and its ability to remain flowable until finally hardened in the baking oven, will produce a wire which is free of faults and uniformly coated.

These two very important features of the present invention I have discovered are due primarily to the use of the solvent in the composition of the present invention, and have resulted in a marked saving in the cost of material, as well as the cost of manufacture, at the same time producing a superior product.

As understood in the art, wire enamels are usually of the oleoresin type including a suitable pigment in the case of the colored enamels, and wherein the oil and resin, which may be natural or synthetic, are cooked together until so combined that they will not separate on cooling, whereupon a suitable solvent for the composition is added.

I have discovered that an excellent solvent for oleoresin bases consists of a hydrogenated petroleum oil obtained commercially from the Standard Oil Company of New Jersey. This solvent is invoiced to Schenectady Varnish Company, Inc. as "Hydrosolvent" and at present numbered in accordance with the boiling range.

This product, I am informed by the Standard Oil Company of New Jersey, is produced in accordance with processes typified by United States patents to Krauch, No. 1,890,434, Dec. 6, 1932, and Pier et al., No. 1,910,050, May 23, 1933, being representative of certain United States and foreign patents owned jointly by it and the I. G. Dye Trust of Germany. Furthermore, I am advised by the Standard Oil Company of New Jersey that this hydrogenated petroleum oil which I utilize as a solvent is a hydrogenation fraction boiling up to 600° F. and is made from a petroleum base. This product is made by the hydrogenation of crude petroleum oils, distillates thereof, cracked petroleum products and other petroleum oils, either crude or in various states of refinement, by the use of high pressure and temperature with or without a catalyst.

The hydrogenation may be carried on to any desired extent, that is, the saturation with hydrogen, and I am also informed that "Hydrosolvent" 110

No. 3" and "Hydrosolvent No. 4", representative of the products manufactured by said Standard Oil Company of New Jersey, have boiling ranges of 365-420° and 420-550° F., respectively, and 5 that similarly produced solvents having a higher or lower boiling range up to 600° F., for example 200-600° F., may be made by the process covered in the patents and patent applications above mentioned.

10 I prefer to use a solvent having a boiling range of between 250° F. and 300° F. to 600° F. In some cases, particularly where the wire is of very thin gauge, a solvent having a boiling range of about 200° F. to 600° F. has been found desirable.

15 I also have discovered that the use of this hydrogenated solvent obtained from petroleum permits more complete oxidation and chemical action of the varnish in the baking chamber and that I secure a hard, permanent, and of particular importance, a non-porous film.

20 Aside from possessing excellent solvent characteristics whereby a film of optimum efficiency is obtained, the hydrogenated petroleum oil solvent is relatively non-evaporative and does not 25 give off fumes which are of the same nature as coal tar derivatives, i. e. benzol or coal tar naphtha, which have a very toxic effect upon the workmen and a very irritating effect on the eyes, nose and throat. The coating prepared with the 30 present solvent on the other hand permits the workmen to operate comfortably with little or no irritation or ill effects.

Furthermore, I find that the use of a solvent 35 of this character is an improvement over the usual coal tar derivative solvents, in that it maintains the stability of the varnish or enamel more acceptably in the usual enameling machines and in the circulating systems used by the large manufacturers to feed these machines. That is 40 to say, the solvent which I have discovered, is effective in maintaining the varnish or enamel free of gelling in the bath and circulating systems, and also in maintaining the coating stable after it has been applied upon the wire before 45 introduction into the usual baking chamber. This will be appreciated, since the solvent is relatively non-evaporative. As stated, the baking of the varnish or enamel takes place at a relatively high temperature and results in a hard, 50 smooth, non-porous and flexible coating thoroughly adherent to the metal base wire.

These various advantages are of particular importance, since I have observed the toxic conditions surrounding the use of coal tar derivatives 55 such as coal tar naphtha, wherein the fumes affect the nose and throat and eyes of the workmen in the enameling room. Furthermore, these coal tar derivatives are not capable of producing the same stability to maintain the varnish constantly in working condition during the various 60 steps leading to the production of the final product. That is, the constant circulation of the enamel or the constant running of the pulleys in the bath over which the wire moves, tends to gell 65 the enamel. With coal tar derivatives this takes place in a relatively short time. The present enamel, however, which includes a hydrogenated petroleum product as above set forth, is relatively non-gelling.

70 In carrying out the present invention, I employ an oil, preferably a vegetable drying oil, or a combination of drying oils. By drying oils, I mean linseed oil, tung oil or perilla oil. In addition, I use in some cases a semi-drying oil such 75 as soya bean oil or fish oil or a non-drying oil,

such as castor oil. These are used alone or suitably combined. The drying and semi-drying oils are glycerol esters of unsaturated organic acids and hence take up oxygen and harden.

75 The resin employed may be a natural one, for example, kauri, or one of the copals. Also, I employ synthetic resins of the cumaron type, the aldehyde condensation product type such as bakelite or the glyptal type, i. e. resins produced from glycerol and organic acids.

80 Both the resins and the oils are well known commercial products and they or their equivalents have been used in the manufacture of varnishes and enamels, so that a specific description of them is not deemed necessary for one skilled 85 in the art.

90 The resin is melted in the usual manner and while in heated condition and fluid, the oil which has previously been heated or blown in another receptacle is added. The oil and resin are cooked together until they are so combined that they will not separate on cooling. Thereupon a suitable quantity of the hydrogenated petroleum solvent referred to above is added and the oleoresin base is dissolved therein. I find that this solvent 95 acts to promote the even dispersion of the base and enhances the flow of the varnish or enamel, since it is relatively non-evaporative and resists gelling. Moreover, and because of these stabilizing characteristics, the varnish is maintained in 100 good working condition and stable in the varnish machines whereby an even coating is applied to the metal wire and which, upon subsequent baking, forms a smooth, hard, but flexible, impervious film. In baking the coated wire, the enamel of the present invention remains stable and fluid until finally set. That is to say, its non-evaporative tendency keeps the enamel from becoming 105 preliminarily hard and porous. The result is then that the enamel is fluid upon the wire in the baking chamber and any potential cracks or gaps in the coating are in effect self-sealed by reason of this continuing fluidity and a smooth continuous coating is produced. The evaporation as 110 explained is gradual, permitting this result and assuring a final, smooth, non-porous, insulating 115 film.

120 In some cases, the varnish or enamel will so react, either due to chemical action and/or the presence of the baking temperature, as to produce 125 a definite color or shade. Thus, for example, I obtain a mahogany color or a purple color without the use of pigments.

130 On the other hand, the trade has indicated a desire for colored enamels and I, therefore, grind the proper pigments, using the wire enamel as a vehicle, and in which the pigment is dispersed, in some cases.

135 The proportions of oil, resin and solvent, of course, will vary with the particular composition being treated, and I make both long and short varnishes and enamels.

140 I use the hydrogenated petroleum solvent alone as the solvent for the oleoresin base or I use mixtures of this solvent, for example, with coal tar naphtha or with a non-hydrogenated petroleum product such as kerosene. The percentage mixtures of the two solvents will be determined by the character of the base.

145 The hydrogenated petroleum solvent is relatively heavy, as will be observed, having a boiling range up to 600° F. and usually of approximately 300-600° F., and I find this of advantage in that not only is the evaporation retarded in the enameling room whereby the condition of 150

the varnish is maintained at optimum efficiency, but, moreover, the vapors are not toxic to the eyes, nose and throat of the workmen as is true of present day solvents derived from coal tar.

- 5 In the case where the solvent has lower boiling ranges below 300° F. as above mentioned, as for example, 200° F., 250° F., or 275° F. to 600° F., the solvent exhibits a similar non-gelling action and self-sealing qualities. The conditions entering into the manufacture of the enamel and its application to the wire are controlled depending upon the nature of the wire, as for example the metal of which it is composed, the gauge of the wire, and the final product desired.
- 10 It is to be understood that in referring to the hydrogenated petroleum oil as a varnish or enamel solvent, I mean as well that it has the function of a thinner or diluent.

15 The varnish is applied to wire, such as copper wire, aluminum wire, nichrome wire, and steel wire, or any other metal wire in a continuous process. That is, the bare wire is on a spool and is run continuously through the bath of enamel and into and through a heating chamber of varying length and the final coated product drawn from the heating chamber is then wound upon another spool. The passage of the wire through the bath and through the heating chamber is controlled, so as to insure a thorough coating and a thorough baking respectively. The baking temperature is usually from 400 to 900° F. In some cases temperatures below 400° F. may be used.

20 The wire removed from the heating chamber and the varnish composition thereon will be found to be chemically changed and completely oxidized into a smooth, hard insulating film thoroughly adherent to the metal wire base and, of particular importance, flexible and free from porosity.

25 A careful examination of the final coating discloses that it possesses novel characteristics as regards adherency to the metal, and particularly as to smoothness, hardness and flexibility. Also, 30 the coating is resistant to the action of solvents and varnishes which are subsequently applied over the coated wire and baked thereon for insulating purposes. Moreover, the coating is of a character to be resistant to temperature changes in 35 use and does not break down in the presence of lubricating oils and cooling liquids under the varying temperature conditions prevailing, for example, where a coil of the wire is used with a transformer.

40 It will be understood that I will, in some cases, combine or mix various of the solvents mentioned to produce a blended solvent; also, that the several solvents having the boiling ranges specified may or may not be of uniform boiling range, and in 45 some cases consist of fractions boiling at the lower ranges specified, as well as fractions which boil at the high ranges.

45 As stated, I make a clear varnish which, upon baking, presents a coating having a suitably colored shade, different from that of the original varnish, or I add to the varnish a suitable pigment for the purpose of producing a desired color. I find that my improved solvent acts to bring out the color very effectively in the clear varnish and is inert with respect to the usual ground pigments.

50 I attribute the very efficient results obtained with the wire enamel of this invention to the advantageous use of the new hydrogenated solvent which, in addition to removing toxic conditions in the manufacturing operation, has the

equally important advantage of materially enhancing the final coating produced upon the wire.

55 This application is a continuation in part of my co-pending application, Serial No. 689,677, filed Sept. 15, 1933.

80

I claim:

1. A wire enamel comprising a drying oil, a resin, and a solvent comprising a hydrogenated petroleum product, which is a hydrogenation fraction boiling from substantially 200° F. to 600° F.

60 2. A wire enamel comprising a drying oil, a resin, and a solvent comprising a hydrogenated petroleum product, which is a hydrogenation fraction boiling from substantially 200° F. to 600° F., and a non-hydrogenated solvent.

65 3. As an article of manufacture, metal wire having baked thereon a wire enamel comprising a drying oil, a resin, and a solvent comprising a hydrogenated petroleum product which is a hydrogenation fraction boiling from substantially 200° F. to 600° F., said enamel being resistant to the action of solvents contained in supplemental insulating coatings and to temperatures employed to bake such insulating coatings over 100 the enamel.

70 4. The process of coating wire which consists in providing a bath of enamel containing a solvent which is a hydrogenated petroleum product boiling between substantially 200° F and 600° F. and which throughout the existence of the bath remains substantially non-evaporative whereby there is provided a substantially permanently non-gelling bath resistant to agitation as occasioned by the continuous passage of a wire length 110 or lengths therethrough, continuously conducting a length of wire through said bath and forming a coating thereon, and setting the coating by subjecting the same to a baking action.

75 5. A wire enamel comprising a drying oil, a resin, and a solvent comprising a hydrogenated petroleum product, which is a hydrogenation fraction boiling from substantially 250-275° F. to 600° F.

80 6. A wire enamel comprising a drying oil, a resin, and a solvent comprising a hydrogenated petroleum product, which is a hydrogenation fraction boiling from substantially 250-275° F. to 600° F., and a non-hydrogenated solvent.

85 7. As an article of manufacture, metal wire having baked thereon a wire enamel comprising a drying oil, a resin, and a solvent comprising a hydrogenated petroleum product which is a hydrogenation fraction boiling from substantially 250-275° F. to 600° F., said enamel being resistant 130 to the action of solvents contained in supplemental insulating coatings and to temperatures employed to bake such insulating coatings over the enamel.

90 8. The process of coating wire which consists in providing a bath of enamel containing a solvent which is a hydrogenated petroleum product boiling between substantially 250-275° F. to 600° F. and which throughout the existence of the bath remains substantially non-evaporative 140 whereby there is provided a substantially permanent non-gelling bath resistant to agitation as occasioned by the continuous passage of a wire length or lengths therethrough, continuously conducting a length of wire through said bath 145 and forming a coating thereon, and setting the coating by subjecting the same to a baking action.

95 9. A wire enamel comprising a drying oil, a resin, and a solvent comprising a hydrogenated petroleum product, which is a hydrogenation 150

fraction boiling from substantially 300° F. to 600° F.

10. A wire enamel comprising a drying oil, a resin, and a solvent comprising a hydrogenated petroleum product, which is a hydrogenation fraction boiling from substantially 300° F. to 600° F., and a non-hydrogenated solvent.

11. As an article of manufacture, metal wire having baked thereon a wire enamel comprising a drying oil, a resin, and a solvent comprising a hydrogenated petroleum product which is a hydrogenation fraction boiling from substantially 300° F. to 600° F., said enamel being resistant to the action of solvents contained in supplemental insulating coatings and to temperatures employed to bake such insulating coatings over the enamel.

12. The process of coating wire which consists in providing a bath of enamel containing a solvent which is a hydrogenated petroleum product boiling between substantially 300° F. and 600° F. and which throughout the existence of the bath remains substantially non-evaporative whereby there is provided a substantially non-gelling bath resistant to agitation as occasioned by the continuous passage of a wire length or lengths therethrough, continuously conducting a length of wire through said bath and forming a coating thereon, and setting the coating by subjecting the same to a baking action.

13. As an article of manufacture, metal wire having baked thereon a wire enamel comprising a drying oil, a resin, and a solvent comprising a hydrogenated petroleum product which is a hydrogenation fraction boiling from substantially 200° F. to 600° F., and a non-hydrogenated solvent, said enamel being resistant to the action of solvents contained in supplemental insulating coatings and to temperatures employed to bake such insulating coatings over the enamel.

14. As an article of manufacture, metal wire having baked thereon a wire enamel comprising a drying oil, a resin, and a solvent comprising a hydrogenated petroleum product which is a hydrogenation fraction boiling from substantially 250-275° F. to 600° F., and a non-hydrogenated solvent, said enamel being resistant to the action of solvents contained in supplemental insulating coatings and to temperatures employed to bake such insulating coatings over the enamel.

15. As an article of manufacture, metal wire having baked thereon a wire enamel comprising a

drying oil, a resin, and a solvent comprising a hydrogenated petroleum product which is a hydrogenation fraction boiling from substantially 300° F. to 600° F., and a non-hydrogenated solvent, said enamel being resistant to the action of solvents contained in supplemental insulating coatings and to temperatures employed to bake such insulating coatings over the enamel.

16. The process of coating wire which consists in providing a bath of enamel containing a solvent which is a hydrogenated petroleum product boiling between substantially 200° F. and 600° F., and a non-hydrogenated solvent, and which throughout the existence of the bath remains substantially non-evaporative whereby there is provided a substantially permanently non-gelling bath resistant to agitation as occasioned by the continuous passage of a wire length or lengths therethrough, continuously conducting a length of wire through said bath and forming a coating thereon, and setting the coating by subjecting the same to a baking action.

17. The process of coating wire which consists in providing a bath of enamel containing a solvent which is a hydrogenated petroleum product boiling between substantially 250-275° F. to 600° F., and a non-hydrogenated solvent, and which throughout the existence of the bath remains substantially non-evaporative whereby there is provided a substantially permanent non-gelling bath resistant to agitation as occasioned by the continuous passage of a wire length or lengths therethrough, continuously conducting a length of wire through said bath and forming a coating thereon, and setting the coating by subjecting the same to a baking action.

18. The process of coating wire which consists in providing a bath of enamel containing a solvent which is a hydrogenated petroleum product boiling between substantially 300° F. and 600° F., and a non-hydrogenated solvent, and which throughout the existence of the bath remains substantially non-evaporative whereby there is provided a substantially non-gelling bath resistant to agitation as occasioned by the continuous passage of a wire length or lengths therethrough, continuously conducting a length of wire through said bath and forming a coating thereon, and setting the coating by subjecting the same to a baking action.

WILLIAM HOWARD WRIGHT.